

Sept. 10, 1929.

J. W. WERRA

1,727,579

NONMARRING HAMMER

Filed May 14, 1927

Fig. 1.



Fig. 3.



Fig. 2.



Fig. 4.



INVENTOR.

BY *Julius W. Werra*  
*Morsell, Kenney & Morsell*,  
ATTORNEYS.

## UNITED STATES PATENT OFFICE.

JULIUS W. WERRA, OF WAUKESHA, WISCONSIN, ASSIGNOR TO WERRA ALUMINUM FOUNDRY COMPANY, OF WAUKESHA, WISCONSIN, A CORPORATION OF WISCONSIN.

## NONMARRING HAMMER.

Application filed May 14, 1927. Serial No. 191,424.

This invention relates to improvements in non-marring hammers as a new article of manufacture.

Non-marring hammers as now used are formed of copper or lead and are objectionable in many respects. Hammers formed of copper or lead are of comparatively small size for their weight, with the result that the force of the blow is applied to a small surface of the material worked on and the surface is marred, fractured, or otherwise injured.

It is one of the objects of this invention to provide a non-marring hammer formed of an aluminum alloy.

In forming the hammer of aluminum, it is necessary to provide for strength, ductility, uniformity, and fineness of grain, structure and toughness, and it has been found that aluminum and 5 to 15 per cent silicon will produce the desired result and form a metal which is relatively soft, and will deform without fracture and has high ductility, fineness of grain and high strength. The ordinary aluminum alloys, such as #12 alloy (8% copper, 92% aluminum) universally used for the general run of castings, such as automotive crank cases, gear cases, etc., have a tensile strength of around 18,000 lbs. per square inch, with 1 1/2% elongation, and Brinell hardness 68 to 72. These castings are comparatively weak, hard and brittle and would fracture after a comparatively few blows. The advantage of an aluminum alloy hammer over a copper hammer is apparent when it is considered that in their comparative specific gravities of 2.56 for aluminum and 8.89 for copper, the aluminum hammer would have 3 1/2 times the surface area, and the advantages over a lead hammer are still more apparent as the specific gravity of 11.37 for lead gives a comparative surface area of 4 1/2 to 1 for the aluminum hammer. Furthermore, as the elasticity of lead is practically nil, greater percentage of a driving blow is therefore effective in working the lead rather than in moving the object driven by the hammer.

It is one of the objects of the present invention to overcome the above mentioned

objectionable features and provide as a new article of manufacture a non-marring hammer formed of an aluminum alloy in which, for a given weight, the striking area of the hammer face is of several times the area of the ordinary hammer.

A further object of the invention is to provide as a new article of manufacture, a non-marring hammer which is comparatively of light weight for its size, is strong and durable, and is well adapted for the purpose desired.

With the above and other objects in view the invention consists of the improved non-marring hammer as a new article of manufacture, and its parts and combinations as set forth in the claims, and all equivalents thereof.

In the accompanying drawing in which the same reference characters indicate the same parts in all of the views:

Fig. 1 is a side view of the improved non-marring hammer;

Fig. 2 is a top view thereof;

Fig. 3 is a rear view of the upper portion thereof; and

Fig. 4 is a front view of the part shown in Fig. 3.

In the drawing, the numeral 5 indicates the handle, which may be formed of wood or any other material desired, and 6 the head which is formed of the improved aluminum alloy. The head is shaped to provide a front flat working portion 7 of rectangular shape, and a rear flat working portion 8 of elongated form. The working faces of the head are more than three times the surface area of non-marring hammers of same weight used in standard practice, so that with a hammer of a given weight, a working surface of more than three times the area of the working surface of a hammer of standard practice is provided, thus distributing the force of the blow on a surface over a greater area.

This hammer is not a sledge hammer, but is in the hand hammer class, in which the mechanician relies rather upon his own muscular effort for the force of the blow and upon the surface area to distribute the force and prevent damage to the object worked, than he

does upon the weight of the hammer, thus permitting the mechanic to better judge the force to be applied and to be more able to direct it.

5. A hammer head formed of the ordinary aluminum alloy, (8% copper and 92% aluminum), which is universally used in making castings, and which would have a tensile strength of about 18,000 lbs. per square inch, 10 with 1½% elongation, Brinell hardness 68 to 72, would be comparatively weak, hard and brittle, and would fracture after a comparatively few blows. To provide an aluminum alloy which will obtain the results desired, the 15 aluminum is mixed with 5% to 15% silicon alloys because of their relative softness, combined with their ability to deform without fracture, their high ductility, fineness of grain and high strength. These alloys range 20 in tensile strength from 15,000 lbs. per square inch with 12% elongation, Brinell hardness 40 for the low silicon (5%) content, to 26,500 lbs. per square inch, with 8% elongation, Brinell hardness 52, for the high silicon 25 (13%) content. The first or 5% alloy is used for hammers for light soft work, while the second or 13% alloy is used for hammers used for hard driving or hard material. In some cases a wider range of percentage of alloys 30 used may be desirable, but in all cases the resultant hammers will have working faces of several times the area of the working faces of standard practice hammers of approximately the same weight.

35. As an example of the differences between the improved hammer and the hammer of standard practice, the improved hammer of one size is formed with a working face of 1¾" x 2" by 5" long, and weighs 1½ lbs. A 40 copper hammer of the same dimensions would weigh 5¼ lbs., and a lead hammer 6¾ lbs.

It will thus be seen that as a new article of manufacture, a non-marring hammer is provided of greater working surface and lighter in weight, and is therefore better balanced than the lead and copper hammers of standard practice, and due to the novel composition used, is still soft, strong and ductile, and 50 is well adapted for the purpose desired.

What I claim as my invention is:

1. As a new article of manufacture, a non-marring hammer formed of aluminum and two to fifteen per cent of silicon alloy to provide a hammer of considerably less weight and a working face of considerably larger area than a corresponding non-marring hand hammer of standard practice, and a handle for said hammer.
60. 2. As a new article of manufacture, a non-marring hammer formed of aluminum and two to fifteen per cent of silicon alloy to provide a hammer of considerably less weight and working faces at its opposite ends of considerably larger areas than a corresponding

non-marring hand hammer of standard practice, and a handle for said hammer.

3. As a new article of manufacture, a non-marring hammer formed of aluminum and an alloy which will toughen the aluminum substantially to the same extent as an alloy of two to fifteen per cent of silicon without increasing the weight substantially beyond what the silicon does to provide a working face of considerably larger area than a corresponding non-marring hand hammer of standard practice, and a handle for said hammer.

In testimony whereof, I affix my signature.

JULIUS W. WERRA.

80

85

90

95

100

105

110

115

120

125

130